

106-97

Cross Reference

Examiner

Feb. 3, 1942.

I. A. NICHOLAS

2,272,018

HOT TOP AND ELEMENT FOR PRODUCING THE SAME

Filed June 30, 1939

2 Sheets-Sheet 1

106  
97

Fig. 1



Fig. 4



Fig. 2



Fig. 3



Fig. 6

Inventor  
Isaac A. Nicholas

George W. Dorn,

Attorneys

SEARCHED  
INDEXED  
FILED  
CROSS REFERENCE

# Cross Reference

Examiner

Feb. 3, 1942.

I. A. NICHOLAS

2,272,018

HOT TOP AND ELEMENT FOR PRODUCING THE SAME

Filed June 30, 1939

2 Sheets-Sheet 2

Fig. 9.



Fig. 7



Fig. 8



Fig. 10



Fig. 11



Inventor  
Isaac A. Nicholas

Bridge Law Firm,

Attorneys

106-97

Patented Feb. 3, 1942

2,272,018

NR

# UNITED STATES PATENT OFFICE

2,272,018

## HOT TOP AND ELEMENT FOR PRODUCING THE SAME

Isaac A. Nicholas, Pittsburgh, Pa., assignor to The Standard Lime and Stone Company, Baltimore, Md., a corporation of Maryland

Application June 30, 1939, Serial No. 282,259

9 Claims. (Cl. 22—147)

This invention pertains to hot tops, which are commonly employed in conjunction with ingot molds to facilitate the filling thereof and to prevent piping and the formation of other defects in the ingot. It is particularly applicable to hot tops for ingot molds in the manufacture of steel.

The hot top of the present invention presents many advantages over the usual hot top now commonly employed, and some of these advantages may be stated generally as follows: lightness of structure, together with compactness in storage; ease of placement with reference to the ingot mold; beneficial effects of the residue of the hot top elements with reference to the mill scale formed as the result of rolling the ingot, along with the production of a high grade ingot substantially free of "hanger cracks" and other surface and interior defects such as voids which are often present under present day practice; and the maintenance of fluidity of the upper portion of the ingot with the result that voids and piping, as well as cropping, are held to a minimum. Other advantages will hereinafter appear.

Most hot tops in use today are formed in whole or in part of fire clay molded to the desired shape and then burned or fired. Such hot tops are heavy and necessitate mechanical equipment and the presence of at least two men to facilitate the placement thereof with reference to the ingot mold. Moreover, when such hot top is stripped or broken away from the ingot, portions of the burned clay will adhere thereto to a greater or less extent due to the metal of the ingot "freezing" to the fire clay. Here, again, manual labor with its attendant expense is essential.

Moreover, it is impossible to remove all of the adherent fire clay from an ingot, so that such adherent portions of the burned clay are carried by the ingot into the blooming mill where they have a deleterious effect upon the ingot and likewise cause roll trouble and contamination of the roll scale, making the scale objectionable for use in an open hearth or a blast furnace charge. On the other hand, the material, or materials, employed to produce the hot top of the present invention have a beneficial effect when used in connection with such charges.

The disadvantages of the hollow fire clay hot top are overcome in part by the use of a hot top consisting of a steel casing lined with fire bricks, which tapers gently upward and which is placed in the top of the ingot mold in the same manner. After the ingot has solidified, this type of hot top can be lifted off the mold. The steel does not

tend to freeze to the fire brick in this mold to the same degree as in the hollow fire clay molds. As the ingot shrinks, due to the tapering shape of the hot top, it tends to pull away from the brick. Yet even in this style of hot top, some fire brick adheres to and contaminates the steel. Offsetting this advantage of shrinkage is the complexity of the hot top itself and its greater clumsiness and weight as compared to a clay hot top. Moreover, a rim of baked fire clay must be placed about the bottom of the steel casing to make a tight joint between the casing and the ingot mold. Again, the fire brick lining of the steel casings must be frequently renewed.

Fire clay mainly is used at the present time in the manufacture of hot tops, either used alone or mixed with a number of substances such as chamotte, coke, limestone, shale, etc. The hot top ingredients are mixed with sufficient water to form a plastic mass which is molded to the desired shape and then fired in a kiln. The resulting product is hard and ordinarily has a crushing strength of the order of 5,000 to 15,000 lbs. per square inch. Up to the present time, it has been considered necessary that a hot top should retain great strength at high temperature, as is the case with fire clay, in order to withstand the pressure of the molten steel. I have discovered that this is not necessary and that a hot top need not have a greater crushing strength than 10 to 15 lbs. per square inch, and may have even less. This is explained by the fact that molten metal solidifies instantly when it touches a relatively cold substance. Thus, in pouring molten metal in a hot top of any composition, the skin of solid steel which immediately forms on the surface of the hot top increases in thickness. This ring or layer of solid steel has sufficient strength to hold within itself a considerable head of molten melt and requires little support from the hot top itself. This discovery has enabled me to produce a hot top composed essentially of basic materials. While the new hot top of my invention has practically little strength and will decompose at high temperatures, nevertheless it has proven to be very satisfactory in actual steel pouring operations and to possess a number of decided advantages over a fire clay-bearing material. The preferred basic materials are magnesium and calcium carbonate, either artificially prepared or occurring in the natural state, and also dolomite.

When molten steel comes in contact with such a hot top, the carbonates will partially decompose. Carbon dioxide gas is driven off, leaving

a powder of magnesium and calcium oxides which have excellent insulating properties. On stripping, most of the hot top material does not stick or adhere to the ingot and the portion remaining on the ingot is readily removed when it comes in contact with the blooming mill rolls. Fire clay hot tops become imbedded in the ingot and the greater portion is not removed upon stripping. When the ingot is rolled, the fire brick is broken away together with the scale which coats the ingot. Ingot scale, or so-called roll scale, is a valuable by-product in steel making. It is a very pure form of iron oxide and is used in blast furnace and open hearth operations. When it is contaminated with fire brick it becomes almost useless, as fire brick is very refractory and is dissolved with great difficulty in a blast furnace or open hearth slag. One of the advantages of this invention is that roll scale if contaminated with the basic materials from which the hot top is made, is improved in its smelting properties.

The excellent insulating property of the basic hot top of this invention is another important advantage. The superiority of magnesia over fire clay brick is well known. The insulating effect of the MgO formed when the hot top decomposes is reflected in an increased yield of sound billets. During a direct test made in a large steel plant extending over a period of four months, it was definitely proven that these basic hot tops furnished an increased yield of sound billets 2% greater than was obtained from ingots poured in a fire clay hot top. An increased yield of 2% in sound billets reflects a saving of approximately thirty cents per ton of steel.

Preferably, the hot top of this invention comprises a plurality of sheets or slabs of insulating material that disintegrate in use, so that the material falls away from the ingot when the ingot is removed from the mold. If any material adheres to the ingot, its composition is such as not to be detrimental to the ingot or the roll scale. The slabs of which the hot top is formed (preferably four in number) fit against the interior faces of the ingot mold and are sustained inside the top of the mold by suitable means in such a way that a part of each of the slabs is inside the mold, and a part of each of the slabs projects above the top of the mold. The projecting portions of the slabs are held in place and reinforced against the weight of the molten metal poured into the mold by wire, metal bands, or a metal casing that fits around the outside of the projecting portions of the slabs, as will hereinafter appear.

The invention is illustrated in the annexed drawings, wherein one of the slabs is shown as well as several means for positioning and maintaining the slabs in place in the upper end of an ingot mold.

In the drawings—

Figure 1 is a top plan view of an ingot mold with a hot top of the present invention positioned in the upper end thereof;

Fig. 2, a transverse vertical sectional view on the line II—II of Fig. 1;

Fig. 3, a perspective view of a further means for holding the slabs of the hot top in place;

Fig. 4, a vertical sectional elevation disclosing a slightly different form of slab positioning and holding means utilizing sustaining hooks and corner clips;

Fig. 5, a fragmentary view illustrating the use

of corner clips alone as the means for holding the slabs in assembled relation;

Fig. 6, a perspective view of one of the slabs with its paper covering (which may or may not be employed) partly removed to expose the slab body;

Fig. 7, a face view of a metallic blank from which a modified form of slab supporting and clamping element is produced;

Fig. 8, a perspective view of said element produced from said blank;

Fig. 9, a top plan view of an ingot mold with the slab-formed hot top positioned and held therein by the utilization of clamps such as shown in Fig. 8;

Fig. 10, a vertical sectional view showing the slab at the left in section, while the slab at the right is in elevation; and

Fig. 11, a perspective view of a portion of the upper part of an ingot mold with two of the slab elements positioned therein and held in place by clamps of the form shown in Fig. 8.

Each of the slabs employed in producing the hot top of the present invention comprises an insulating material of light weight, a reinforcing material and a binder, the slab being so made as to provide a porous body of greater insulating value than the fire clay and fire brick hot tops. The hot top insulation keeps the top of the ingot soft and mobile longer than the hot tops now in use and prevents or greatly reduces the formation of voids and piping in the ingot.

The following is one example illustrative of the practice of this invention in the production of the slabs: A magnesia containing lime produced by burning a dolomite with a low percentage of impurities is treated with water to remove enough of the lime to produce an insoluble residue which on an ignited basis has about the following composition:

|                                                  | Percent |
|--------------------------------------------------|---------|
| MgO                                              | 89      |
| CaO                                              | 10      |
| R <sub>2</sub> O <sub>3</sub> + SiO <sub>2</sub> | 1       |

45 This insoluble magnesia-containing sludge is carbonated, whereby a finely divided precipitate is obtained comprising the corresponding amounts of magnesium carbonate and calcium carbonate. To the finely divided carbonates are added wood shavings and starch, and the aggregate is mixed with water to form a moist pasty mass. The proportions in which the ingredients are mixed are approximately as follows:

|               | Parts by weight |
|---------------|-----------------|
| Carbonates    | 89              |
| Wood shavings | 5               |
| Starch        | 6               |
| Water         | 20              |

60 The mixture is pressed into slabs under a pressure of 6 lbs. per square inch. The slabs are placed in a dryer and dried until the water content is not in excess of 1%. I have found that the temperature required so to reduce the water content of the slabs varies with different materials and that the minimum temperatures required range from about 200° C. to about 370° C. The dried slab is a porous mass of sufficient strength to withstand shipping and handling both in storage and in use.

When the composition of the slab is such that the temperature required to reduce the water content to less than 1% is high, the heat impairs the strength of the reinforcing constituent, if wood shavings and other combustible fibrous

materials are used as the reinforcing constituent, as in the preceding example. Under such conditions it is preferable to use a reinforcing constituent that is not affected by the drying temperature. Certain inorganic and non-combustible fibrous and matted materials such as steel wool and steel shavings are unaffected by the highest drying temperatures required and retain their original strength during the drying process, and at the same time do not introduce any constituents that would contaminate or be deleterious either to the ingots or to the roll scale.

The following is one example of the practice of this invention in the production of the slabs, wherein the reinforcing constituent is steel wool and the binder is Portland cement. The basic carbonate constituent is prepared as a slurry containing about 17 to 20% of solids by mixing that constituent with water. To 76 to 88 parts by weight of this slurry are added 4 parts by weight of high early strength Portland cement, and 1 part by weight of steel wool, and the ingredients mixed to thoroughly distribute them. This mixture is run into molds and sufficient water removed, either by squeezing it out under pressure or sucking it out under partial vacuum, to convert it to a thick paste. The material in the molds is then subjected to a pressure of about 400 to 450 pounds per square inch to produce a slab that can be removed from the molds. These slabs are dried to reduce their water content to less than 1% in the manner described in the preceding example.

The composition of the dried slabs is approximately:

|                  | Per cent |
|------------------|----------|
| Basic carbonates | 75       |
| Steel wool       | 5        |
| Portland cement  | 20       |

The slabs will be made of such size as to conform to the usual measurement of the ingot molds. Generally stated, two sizes of slabs are made, one 23x15x1½", and the other 17x15x1½", the smaller slabs weighing about 7 lbs. each, and those of the larger size about 8 lbs. The slabs necessary to produce the hot top have an aggregate weight of approximately 35 lbs., as compared to a weight of approximately 200 lbs. and more of the commercial hot tops of today. The actual weight of the slabs will, of course, vary with variations in porosity and is dependent upon the composition of the slab. The preceding weights are cited by way of illustration and not by way of limitation. The slabs may be stacked and closely packed, both in shipment and in storage, and take up about only one-fifth the space required to store an equivalent number of fire clay hot tops.

As above noted, various means may be employed to maintain the slabs in position in the upper end of the ingot mold. Referring to Figs. 1 and 2, 10 denotes the ingot mold or the upper portion thereof, and 11 denotes the various slabs positioned and maintained within the upper portion or mouth of the mold. In these two figures, hooks 12 are employed, the upper ends of which overlie and embrace the upper edge of the ingot mold, while the lower ends are also hook-shaped and extend under and slightly upward of the lower portion or edge of the slabs 11. As will be seen more particularly upon reference to Fig. 2, the upper portions of the slabs extend upwardly beyond the upper edge of the mold and likewise

extend a somewhat greater distance inwardly of the mold. As shown in Fig. 1, one end of each of the slabs is slightly rounded or contoured to fit the filleted corner of the ingot mold, while the opposite end of the slab is straight and takes against the inner face of the adjacent slab. Thus, the slabs are in a sense interlocked and inasmuch as they are made to size or approximately so, they may be readily positioned within the mold and held in place through the assistance of the sustaining hooks.

In Fig. 3, the upper ends of the slabs which project beyond the ingot mold are embraced by a metallic frame comprising a plurality of plates 13, each end of each plate being out-turned at an angle of approximately 45 degrees to its body, so that adjacent ends of adjacent plates stand in parallelism and are provided with openings through which bolts or screws 14 may be passed to hold the parts in their assembled position.

In Figs. 4 and 5, a still further modification is shown, wherein hooks 12, similar to the hooks shown in Figs. 1 and 2 and so lettered, are employed. Placed at each of the corners of the upwardly projecting portions of the slabs 11 is what may be termed a clip, designated by 15, produced from sheet metal bent upon itself at right angles and fitting against the adjacent ends of the various slabs. These clips are held in position by a wire 16 passed about the assembly and twisted at its ends.

A slab is shown in perspective in Fig. 6. As seen in that view, the slab is provided with a covering 17 of relatively impervious paper or like material which to a certain degree acts as a reinforcing element and has the additional advantage of protecting the slab against the absorption of moisture. This covering will burn away immediately the molten metal contacts the same and, therefore, does not militate against the porosity of the slabs. This is a feature of some importance. It will be appreciated that by reason of the nature of the formation of the slabs, they may be trimmed if need be, to secure proper positioning thereof within the ingot mold.

In Figs. 7 to 11, inclusive, a further modified form of slab supporting and clamping means is illustrated. As will be seen upon reference to Fig. 7, the blank when cut out takes substantially the form of the letter H, with the body portion 20 above the cross-bar or connecting element 21 left integral therewith. The blank may be said to comprise a body 20, the base of which is the full width of the blank with two depending legs or elements 22 and 23 and two upstanding arms or elements 24 and 25, formed by slitting the blank vertically. The body 20 is bent at right angles upon a medial line, while the legs 22 and 23 at their lower ends are bent inwardly and thence upwardly to produce hooks 26 and 27. The arms 24 and 25 are bent outwardly at right angles, as best indicated in Fig. 8, and thence downwardly, producing hook-shaped elements 28 and 29. When positioned within the top of the ingot mold and in proper relation to the slabs, the arms 24 and 25 overlie the upper edge of the ingot mold, while the body 20 embraces the adjacent faces of the slab elements.

The slabs are supported by the hooks 26 and 27 formed upon the lower ends of the leg elements 22 and 23, so that the slabs are precluded from dropping downwardly into the ingot mold. When the clamps or clips are mounted at each corner of the mold and in engagement therewith and with the slabs as just indicated, the slabs

will be quite firmly held in place, the body 20 embracing the corners and the arms and hooks holding the slabs against movement both vertically and laterally.

If desired, a wire 29 may be passed around the upper portion of the assembled slabs or hot top elements and the body 20 of the clips, as shown in Figs. 9 and 11, the wire being twisted to draw the parts into close relationship.

By making the parts integral and having the body portion 20 contact the abutting and adjacent slabs, a stable positioning of the parts is ensured and facility of placement is simplified over the forms previously set forth.

From the foregoing, it will be seen that the clamps or clips may be formed from a single piece of metal by a simple operation of slitting or cutting, and then bending the parts to position. They may be said to comprise a body portion adapted to embrace the adjacent corners or edges of the two slabs, plus hooks to engage the lower edges of the adjacent slabs and supporting arms which overlie the upper marginal end of the ingot mold.

The use of clips or holders of the type just set forth facilitates the positioning of the slabs with reference to the ingot mold and requires the use of only four clips, whereas in the form shown in Figs. 1 and 2 eight are required, and in the form of Fig. 4 twelve are needed. Moreover this form greatly reduces the time and labor required in positioning the insulating slabs to form the hot top.

Any suitable supporting and positioning means may be employed, although in actual practice it has been demonstrated that the style of holder illustrated in Figs. 7 to 11, inclusive, is far superior to any other type of holder so far devised.

The insulating material which comprises the dominant constituent of the slab may be magnesium carbonate, calcium carbonate, a mixture of magnesium and calcium carbonates in any desired proportions, or any other suitable inert insulating material that will not react with the metal being cast. It is essential that the slabs have adequate strength to permit handling and placement of the same but, on the other hand, they should be so produced that they will disintegrate when subjected to the heat of the molten metal, and that the constituents of which the slab is produced will not be detrimental to the ingot or the roll scale.

The reinforcing material used to hold the slab constituents together and to afford sufficient strength and a certain degree of flexibility, may be wood shavings, excelsior, cellulose fibre or any other fibrous and matted organic or combustible substance, or it may be steel wool, steel shavings or any other fibrous or matted inorganic substance which is free of ingredients that would be detrimental to the ingots or the roll scale.

The reinforcing of the slab need not be imparted entirely or even in part by an interior matted fibrous substance, but may be applied exteriorly to the surface of the slab, provided it be of such a nature as not to interfere with the disintegration of the slab when it is heated in contact with the ingot. Exteriorly applied reinforcing covering the faces of the slab has the additional advantage of protecting the slab from the absorption of moisture, and thereby reduces the tendency to boil.

The cementitious material or bond may be starch, glue, sodium silicate, Sorel cement, gypsum, Portland cement or any other cementing

medium that will serve to form a consolidated slab. Preferably, the binder should have the property of disintegrating when subjected to the heat of the molten metal within the time that the ingot remains in the mold.

After the hot top is formed by placement of the slabs in the upper end of the ingot mold, the molten metal is poured through the hot top and passes down into the mold. When the insulating constituent of the slab is composed of carbonates of magnesia and lime in substantially the proportions above specified, the heat of the molten metal will transform the carbonates into oxides that are highly refractory and prevent the transmission or dissipation of heat therethrough. It follows, therefore, that the top of the metal of the charge remains molten for a considerable period of time and much longer than with the hot tops now in commercial use. In a specific case, the surface remained molten forty minutes when hot tops of the present invention were used, and only twenty-nine minutes when fire clay hot tops were employed, and the average sinkage of the top of the metal was 5 inches with the new hot top as compared with 3.7 inches with the clay top, indicating the filling of more voids in the ingot when using the new top. The prolongation of the freezing time of the top of the ingot may be greater or less than in this case, depending on the insulating qualities of the slabs and on other variable conditions. In any event, due to the superior insulating qualities of these slabs, the freezing of the top of the ingot is delayed long enough to allow more time for the molten metal at the top to sink in the mold as the ingot shrinks, and fill the space that would otherwise develop as pipes and voids. Due to the heat of the molten metal, the slab disintegrates in about 15 to 20 minutes, without reacting with the metal.

It is recognized that the time required for the disintegration of the slab varies, depending on the thickness, the density and the composition of the slab. However, when the ingot is removed from the mold, in about an hour, the disintegrated material falls away of itself. If, perchance, any of the material does adhere to the ingot its composition is such as not to be detrimental to the roll scale. The resulting roll scale is, consequently, uncontaminated by objectionable material derived from the hot top.

The invention is not to be restricted to a particular method of making the slabs. They may be made by molding, pressing or extruding, or any other method which will produce a slab. The pressure used in molding should not be great enough to impair the porosity of the slab or to make it so dense as to render its adequate drying difficult.

Moreover, the invention is not to be restricted to a particular temperature or duration of time of drying. Care must be exercised, however, in drying the slabs in order not to impair their strength and make them brittle. Too rapid drying and drying at too high a temperature both have a tendency to make the slabs brittle and result in loss from breakage. The drying may be carried out in any manner that will produce a slab having the requisite strength and that will not boil when subjected to heat of the molten metal. Both in transportation and storage the slabs should be protected against moisture, which would tend to cause boiling when in use.

In its broadest aspect this invention pertains to a hot top which comprises a consolidated mass of insulating material that disintegrates when

subjected to a high temperature and which is of such composition that it will not contaminate the roll scale with objectionable matter. Though the invention has been described in terms of a hot top formed from slabs, the application of the invention is not limited to such slab construction, but includes hot tops consisting of a single unit and molded forms.

What is claimed is:

1. A hot top for ingot molds, comprising a plurality of separate slabs each composed in the main of a finely divided basic inorganic heat insulating material, and a cementitious binding substance for holding the basic material together, said hot top being characterized by the property of disintegrating to a powdery mass of non-adherent particles when subjected to the heat of the molten metal teemed into the mold to produce an ingot.

2. As a new article of manufacture, an insulating slab comprising an admixture of the following: magnesium and calcium carbonate, a fibrous substance, and at least one binding substance, said carbonates forming the major portion of the slab, said slab being characterized when subjected to the temperature of molten metal by the absence of boiling and the ultimate disintegration of the slab as a whole into non-adherent particles.

3. A hot top element for ingot molds, comprising 89 parts by weight of finely divided magnesium and calcium carbonates, 5 parts by weight of wood fibre, and 6 parts by weight of starch, said element being characterized by the property of disintegrating when subjected to the heat of the molten metal teemed into the ingot mold.

4. A hot top for ingot molds, comprising in the main a basic inorganic insulating material combined with a reinforcing material and a cementitious binder, said hot top having the property of disintegrating when subjected to the heat emanating from the metal teemed into the mold to produce an ingot.

5. A hot top for ingot molds, comprising in the main at least one basic carbonate combined with a relatively small amount of steel wool as a reinforcing material and a cementitious binder, said hot top having the property of disintegrat-

ing when subjected to the heat emanating from the metal teemed into the mold to produce an ingot.

6. A slab for use in the formation of a hot top for ingot molds, said slab comprising predominant amounts of the carbonates of magnesium and of calcium, a relatively small amount of fibrous strengthening material, and a binding material likewise present in a relatively small amount, said slab being characterized by being porous, light in weight, and having the property of disintegrating to a powdery mass of non-adherent particles under heat from the molten metal.

10 7. A slab for use in the formation of a hot top for ingot molds, said slab comprising predominant amounts of finely divided carbonates of magnesium and of calcium, a relatively small amount of combustible fibrous strengthening material, and a relatively small amount of starch serving to bind the various carbonate elements together when subjected to light pressure, said slab being characterized by being porous, light in weight, and having the property of disintegrating to an amorphous mass of non-adherent particles under heat.

20 8. A slab for use in the formation of a hot top for ingot molds, said slab comprising predominant amounts of finely divided carbonates of magnesium and of calcium, a relatively small amount of steel wool, and a relatively small amount of Portland cement serving to bind the various carbonate elements together when subjected to pressure, said slab being characterized by being porous, light in weight, and having the property of disintegrating to an amorphous mass of non-adherent particles under heat.

30 9. A hot top element, comprising 75 parts by weight of finely divided magnesium and calcium carbonates, 5 parts by weight of steel wool, 20 parts by weight of Portland cement, and water, said ingredients being admixed, molded, and dried, said element being characterized by the property of disintegrating when subjected to the heat of the molten metal introduced into the mold.

ISAAC A. NICHOLAS.